

## UNITED STATES PATENT OFFICE

2,388,257

## BODIED OIL AND METHOD

Otto Eisenschiml and Gerald Eisenschiml, Chicago, Ill., assignors to Otto Eisenschiml, Bertha J. Eisenschiml, Gerald Eisenschiml, and Rosalie Eisenschiml Gingiss, doing business as a partnership under name The Scientific Oil Compounding Co., Chicago, Ill.

No Drawing. Application May 10, 1941,  
Serial No. 392,940

11 Claims. (Cl. 106—222)

This invention relates to an improved bodied oiticica oil and to the method of making it; it also relates to varnishes made from this bodied oil.

It has long been a problem in the varnish-making art to provide a relatively inexpensive substitute for China wood oil. Oiticica oil is a relatively inexpensive drying oil that has been used heretofore in lieu of China wood oil; however, its use has not been very successful because it does not have the desired quick-bodying characteristics of China wood oil. Varnishes formed from this oil are objectionable from a cost standpoint because they can be thinned only to a limited extent with thinners and because the films deposited from these varnishes are non-elastic and brittle off readily from surfaces on which they are formed. In addition, these oiticica oil varnishes do not dry rapidly and do not have certain other desired physical characteristics such as spread and flow.

We have found that oiticica oil can be treated in accordance with our invention and that the resulting treated oil will body in the kettle at least as fast as China wood oil and even faster, as desired. Moreover, the treated oil of our invention, when used in a varnish, will produce a film similar to China wood oil in drying and elasticity and which has none of the objectionable brittleness characteristic of films formed from untreated oiticica oil-containing varnishes.

In carrying out our invention, oiticica oil is heated in a suitable vessel, for example, a steam-jacketed kettle, to a temperature in the order of about 325° F. to 370° F., preferably about 350° F., and held at approximately that temperature for about ½ hour to 2 hours. Throughout the heating interval, air from any suitable source of supply is introduced into the body of oil from a jet or nozzle or other air distributing device located, preferably, at or adjacent the bottom of the vessel. The effectiveness of contact between the oil and air may be augmented by mechanical agitation, if desired, in which case the kettle may be provided with an agitator. The amount of air bubbling through the body of heated oil may be varied rather widely to meet any desired requirement in the treated oil; however, for most purposes, the introduction of air at the rate of about 2 cu. ft. per minute for each 100 lbs. of oil is sufficient. This combined heat and air treatment is continued until the desired bodying qualities are obtained. This can be determined experimentally by making gelation tests of samples from the kettle from time to time. In most instances, the de-

sired bodying qualities are obtained in from about 30 to 80 minutes.

The heat- and air-bodying treatment of our invention may be carried out in the presence of 5 catalysts. Examples of suitable catalysts are zinc oleate, zinc resinate, manganese oleate and the like as well as salts of nickel, cobalt, lead, iron and the like, and finely divided metals such as zinc dust and the like.

10 By operating in accordance with our invention, fast-bodying oiticica oils may be obtained with a Worstell test of about 4 to about 7 minutes, as desired, as compared with China wood oil, the standard, with a Worstell test varying from about 15 to 8 minutes. The heat- and air-bodied oiticica oils may be cooked into a varnish much like China wood oil, but the cooking temperature need not, and, preferably, should not, exceed about 460° F. and, in some cases, may be as low as about 400° F. 20 On the other hand, China wood oil is usually cooked into a varnish at a temperature in the order of about 560° F. Varnishes made in accordance with our invention are as gas-proof as China wood oil varnishes. Where rosin, modified phenolic condensation products and like resins are used along with the bodied oiticica oil in a varnish, the films formed are gas-proof, even though the varnish is free from driers.

25 The gelation characteristics of the heat- and air-bodied oiticica oils of our invention and the characteristics of the resulting gel are substantially identical with China wood oil as is evident from the results obtained by subjecting a sample of our bodied oiticica oil to the Worstell heat test, as follows: 150 gms. of oil of our invention was heated in an open container to a temperature of 540° F. in 4 minutes while stirring with a thermometer. The heated oil was held at this temperature and the stirring was continued until the 30 oil gelled solid. This took slightly more than 4 minutes. As in the case of pure China wood oil which has been similarly treated, but which requires a holding period of from about 6 to 8 minutes for solid gel formation, the resulting gel was dry, non-adherent to a spatula when cut and crumbly under the pressure of the spatula without sticking. The cut portions crumbled under pressure like dry bread crumbs.

35 40 45 50 55 For purposes of comparison, untreated oiticica was also subjected to the Worstell test. The heated oil was held at 540° F. for in excess of 15 minutes before what could be termed a solid gel was formed. The gel, however, was soft and sticky and would not crumble, and, in general,

resembled the gel formed from adulterated China wood oil.

The following is an example of a mixing varnish made from a treated oiticica oil in accordance with our invention. It is to be understood that the details of the illustrative example may be varied widely to meet any desired need in a varnish without departing from the scope of our invention:

|                               |          |     |
|-------------------------------|----------|-----|
| Limed rosin-----              | lbs.     | 100 |
| Treated oiticica oil-----     | gals.    | 30  |
| Mineral spirits-----          | gals.    | 60  |
| 10% zinc naphthenate-----     | liq. oz. | 25  |
| 6% cobalt naphthenate-----    | liq. oz. | 50  |
| 6% manganese naphthenate----- | liq. oz. | 10  |

The varnish was prepared by cooking the rosin and treated oiticica to a temperature of about 460° F. and holding it at this temperature to a pill body. The driers were added, the varnish cooled, and then thinned with the mineral spirits.

This varnish cooked to a desirable heavy body, fairly low solid content (46% solids), and good retention of elasticity. Films of this varnish dried quickly forming a water-proof and gas-proof, elastic film which exhibited no tendency to brittle off even after long exposure in the open. A similar varnish made with untreated oiticica oil for comparative purposes was low in viscosity and the resultant film was not much better than gloss oil and shortly exhibited a tendency towards brittling off.

One or more of the driers of the above-illustrative varnish formula may be replaced with other suitable driers or omitted, if desired. The limed rosin may be replaced by ester gum, or by kauri gum, sandarac, dammar and like natural resins, or by synthetic resins such as, for example, the phenolics sold under the trade names "Durez," "Lewisol 320," "Beckacite 1101," or by any desired mixture of resins to meet any desired need in a varnish. In the case of ester gum varnishes in accordance with our invention, it is advisable to use driers therein in the event a completely gas-proof varnish film is desired. The mineral spirits may be replaced by other suitable diluents such as V. M. & P. naphtha and the like, or by any desired mixture of diluents.

Another illustrative mixing varnish in accordance with our invention may be prepared as follows: 100 lbs. of ester gum are mixed in a kettle with 25 gals. of treated oiticica oil and are heated to 460° F. and held at that temperature for about 40 minutes. The varnish base is permitted to cool and is then thinned with 55 gals. of mineral spirits, 32 liq. oz. of 10% zinc and 32 liq. oz. of 6% cobalt.

The bodied oil of our invention may be used for other purposes than for the preparation of varnishes. Thus, it may be used in paints, inks and other coating compositions, and, in general, in lieu of China wood oil wherever China wood oil has been used heretofore.

We claim:

1. The method of treating oiticica oil to convert the said oil into a fast-bodying oil having a Worstell test of about 4 to about 7 minutes thereof comprising, heating a body of oiticica oil to a temperature in the order of about 350° F. and holding it at about that temperature for a period of from about one-half hour to about two hours while intimately contacting the heated oil throughout the body thereof with air.

2. The method of treating oiticica oil to con-

vert the said oil into a fast-bodying oil having a Worstell test of about 4 to about 7 minutes thereof comprising heating oiticica oil to a temperature in the order of about 350° F. and holding it at about that temperature for a period of from about one-half hour to about two hours while bubbling air through the heated oil.

3. The method of treating oiticica oil to convert the said oil into a fast-bodying oil having a Worstell test of about 4 to about 7 minutes thereof comprising heating oiticica oil to a temperature in the order of about 350° F. and holding it at about that temperature for a period of from about one-half hour to about two hours, and simultaneously bubbling air through the heated oil throughout the heating period.

4. The method of treating oiticica oil to convert the said oil into a fast-bodying oil having a Worstell test of about 4 to about 7 minutes thereof comprising heating oiticica oil to a temperature in the order of about 350° F. and holding it at about that temperature for a period of from about 30 to 80 minutes and simultaneously bubbling air through the heated oil.

5. The method of treating oiticica oil to convert the said oil into a fast-bodying oil having a Worstell test of about 4 to about 7 minutes thereof comprising heating oiticica oil to a temperature in the order of about 350° F. and holding it at about that temperature for a period of from about 30 to 80 minutes and simultaneously bubbling air through the heated oil throughout the heating period.

6. The method of treating oiticica oil to convert the said oil into a fast-bodying oil having a Worstell test of about 4 to about 7 minutes thereof comprising heating oiticica oil to a temperature in the order of about 350° F. and holding it at about that temperature for a period of from about 30 to 80 minutes and simultaneously bubbling air through the heated oil throughout the heating period at the rate of about 2 cu. ft. per minute for each 100 lbs. of oil being treated.

7. A heat- and air-bodied oiticica oil capable of being cooked into a varnish at a temperature of about 400° F. to 460° F. and having a Worstell test of about 4 to 7 minutes, said oil having been prepared substantially in accordance with the method of claim 1.

8. A heat- and air-bodied oiticica oil capable of being cooked into a varnish at a temperature of about 400° F. to 460° F. and having a Worstell test of about 4 minutes, said oil having been prepared substantially in accordance with the method of claim 2.

9. A heat- and air-bodied oiticica oil capable of being cooked into a varnish at a temperature of about 400° F. to 460° F. and having a Worstell test of about 7 minutes, said oil having been prepared substantially in accordance with the method of claim 2.

10. A varnish comprising the cooked reaction product of a resin and a bodied oiticica oil having a Worstell test of about 4 to 7 minutes which has been prepared substantially in accordance with the method of claim 2.

11. A varnish comprising the product formed by reacting a bodied oiticica oil having a Worstell test of about 4 to 7 minutes and which has been prepared substantially in accordance with the method of claim 2 with a resin to a pill body at a temperature of about 400° F. to about 460° F.

OTTO EISENSCHIML.  
GERALD EISENSCHIML.

CERTIFICATE OF CORRECTION.

Patent No. 2,388,257.

November 6, 1945.

OTTO EISENSCHIML, ET AL.

It is hereby certified that error appears in the printed specification of the above numbered patent requiring correction as follows: Page 2, first column, line 68, same page, second column, lines 3, 11, 19-20, 28 and 37, strike out the word "thereof"; and that the said Letters Patent should be read with this correction therein that the same may conform to the record of the case in the Patent Office.

Signed and sealed this 5th day of February, A. D. 1946.

Leslie Frazer

(Seal)

First Assistant Commissioner of Patents.